

## UNITED STATES PATENT OFFICE

2,652,369

LIQUID ADDITION PRODUCT OF AN ACETAL  
AND DIALKYL ESTERS OF AN ALPHA-BETA  
UNSATURATED ALIPHATIC DICARBOXYL-  
IC ACID AS AN ANTIFOAMING AGENT FOR  
HYDROCARBON OILSJoseph E. Fields, Dayton, Ohio, assignor to Mon-  
santo Chemical Company, St. Louis, Mo., a cor-  
poration of DelawareNo Drawing. Application November 27, 1950,  
Serial No. 197,837

3 Claims. (Cl. 252—56)

1

This invention relates to antifoaming hydrocarbon oils and deals more particularly with hydrocarbon oils containing as antifoaming agents, small amounts of certain ketonic esters.

The problem of foam inhibition is one of major importance to all industries employing hydrocarbon oils under foam-inducing conditions. While most oils will foam to some extent due to vigorous agitation and aeration in a running engine, foaming becomes a problem only when loss of oil occurs by foam seepage or when so many air bubbles are present in the oil that proper lubrication of bearing surfaces is impeded. Foaming is often experienced with dry sump engines in which there is employed a scavenger pump for collecting oil from various engine parts and returning it to the lubricant reservoir. Here air may be collected along with the oil and deposited in the reservoir. The design and operation of aircraft engines is such that foaming occurs more readily in this type of engine than it does in automotive engines.

Foam and froth in hydrocarbon oils, however, is not due solely to engine design although location and design of the oil pump, oil sump and oil lines as well as modification of other mechanical features may retard foam development; when certain oils are employed with high speed engines, mechanical control, alone, does not suffice. Here, the nature of the crankcase oil is often the prime factor in foaming difficulties. The heavier the grade of the oil or the higher the viscosity of the oil, the more difficult it is to avoid foaming. Heavy grade oils, such as those employed in high-speed diesel and spark ignition engines operating under severe conditions are particularly susceptible to foaming. The heavy oils hold bubbles very firmly so that when foam is formed, it is very persistent.

New developments in engine construction have constantly demanded lubricants having properties not possessed by crude hydrocarbon oils. Such properties are now generally imparted to lubricants by the use of additives. For example, in order to satisfy the lubrication requirements of hypoid gears, materials which impart extreme-pressure resisting properties are now generally added to gear lubricants. In most cases, however, the improvement attained in oils by the use of additives is made only at the expense of increasing its susceptibility to foam. Thus, while the demands of modern engine design for extreme pressure resisting lubricants, for anti-

2

corrosive lubricants, for lubricants of increased viscosity and low-pour-point and good detergents properties have been met by the formulation and use of numerous chemicals which give these desirable properties to oils when admixed therewith, the use of such additives makes the treated oils particularly susceptible to foaming. While light grade oils, e. g. SAE 10 grade oils, are almost non-foaming under the most severe conditions, when there are employed with these oils one or more additives such as viscosity index improvers, extreme pressure resisting improvers, pour-point depressors, etc., the resulting "improved" oils do not retain their non-foaming characteristics and are frequently even more susceptible to foaming than are the heavy grade oils.

Hence, with the development of new high-speed engines and the provision of the new additive-type lubricants, the problem of foaming has assumed major importance. Attempts to solve the problem by defoaming existing oils, e. g., by submitting oils to heat-treatment, absorption processes, filtering steps, etc., have proved of but little value. The most practical solution to this problem has been made by the use of antifoam additives.

A number of antifoam additives, i. e., antifoaming agents, foam depressing agents, foam depressants, antifrothers or foam suppressors, are known; but in the prior art their use has been attended with numerous difficulties. Among disadvantages of such known additives are chemical reactivity with the lubricant or other oil additives, corrosive effect, susceptibility to decomposition upon heating, instability when exposed for long periods of time to ordinary atmospheric conditions, high cost, etc.

Now I have found that foaming of hydrocarbon oils is efficiently retarded and even completely inhibited when there is added to such oils a small quantity, say, from 0.001 per cent to 1.0 per cent by weight of a liquid addition product of one mole of an acetal with from 2 to 20 moles of certain dialkyl esters of an alpha-beta unsaturated aliphatic dicarboxylic acid of not more than 6 carbon atoms. Addition products of this kind are described in the copending application of Tracy M. Patrick, Serial No. 197,829, filed of even date. They are readily obtained by contacting an acetal having the general formula shown below with the dialkyl dicarboxylate in the presence of a free-radical liberating agent

and maintaining the resulting mixture at ordinary or increased temperatures until formation of a liquid mixture of addition products has been formed and separating any unreacted material and 1:1 molar addition product from the resulting reaction product. The residue thus obtained consists of a mixture of a series of adducts. Each adduct contains only one mole of the acetal, but the number of moles of ester present in each adduct may be from 2 moles to 10 20 moles of ester per mole of acetal. The individual adducts present in the mixture may be separated from each other only with difficulty; for the present purposes the liquid mixture of adducts is employed.

Free-radical-liberating catalysts employed in preparing the liquid mixture of adducts are for example inorganic or organic peroxidic compounds such as acetyl peroxide, t-butyl peroxide, t-butyl hydroperoxide, benzoyl peroxide, lauroyl peroxide, stearoyl peroxide, hydrogen peroxide, peracetic acid, sodium perborate, potassium persulfate and the like. Instead of the peroxidic catalyst, ultra-violet radiation may be employed.

Acetals employed for the preparation of the present liquid addition product have the general formula



wherein R is selected from the group consisting of hydrogen, alkyl, cycloalkyl and aralkyl radicals, and R' and R'' are saturated hydrocarbon radicals. Preferably R is an alkyl radical containing up to 7 carbon atoms. R' and R'' preferably contain up to 7 carbon atoms and more preferably are identical alkyl radicals.

The term "saturated" as used herein excepts normal benzene ring unsaturation since benzene does not give any reaction with bromine water and practically all of its reactions are those of substitution instead of addition.

Illustrative acetals are, for example,

Dimethoxymethane  
Diethoxymethane  
1,1-dimethoxyethane  
Acetal (1,1-diethoxyethane)  
1,1-diethoxybutane  
1,1-diethoxyheptane  
1,1-dipropoxyheptane  
1,1-dibutoxyethane  
1,1-(di-2-ethylhexoxy)butane  
1,1-didodecoxydodecane  
1-methoxy-1-ethoxyethane  
1-propoxy-1-butoxybutane  
1,1-dicyclopropoxyheptane  
1,1-dicyclohexoxybutane  
1,1-dibenzyloxyethane  
1,1-diphenethoxybutane  
1,1-diphenoxyheptane  
1,1-ditolyloxybutane  
1-ethoxy-1-cyclohexoxypropane  
1-benzoyloxy-1-phenoxylhexane  
1-cyclopropoxy-1-tolyloxypentane  
1-ethoxy-1-phenethoxyethane  
Diethoxycyclohexylmethane  
Dibutoxycyclopropylmethane  
1,1-dimethoxy-2-phenylethane  
1,1-dipropoxy-2-tolylethane  
and the like

Dialkyl  $\alpha,\beta$ -aliphatic olefinic dicarboxylates

used for the preparation of the present anti-foaming agents have the general formula



in which Y and Z are selected from the class consisting of hydrogen and the methyl radical and X is an alkyl radical of from 1 to 8 carbon atoms. Examples of useful dialkyl carboxylates having the above general formula are dimethyl, diethyl, di-n-butyl, diisobutyl, di-tert-butyl, di-n-amyl, diisoamyl, di-tert-amyl, dihexyl, diisohexyl, di-in-heptyl, and di-n-octyl, maleates, fumarates, citraconates and mesaconates.

The present liquid addition products may be represented by the formula



in which R is selected from the class consisting of hydrogen, alkyl, cycloalkyl and aralkyl radicals, R' and R'' are saturated hydrocarbon radicals, Y and Z are selected from the class consisting of hydrogen and the methyl radical, X is an alkyl radical of from 1 to 8 carbon atoms and n is an integer of from 2 to 20.

The present acetal-ester adducts are effective antifoaming agents when they are employed in very low proportions, i. e., in amounts of up to 1.0 per cent by weight, based on the weight of the total hydrocarbon oil composition. From 0.01 per cent to 0.5 per cent of the adducts is preferred, depending upon the nature of the oil. Heavy oils and oils containing foam-inducing adjuvants require more of the present anti-foaming adducts than do base oils of good viscosity characteristics.

The antifoaming effect of the acetal-ester adducts is not materially affected by the presence of other adjuvants in the oil. The present adducts are stable materials which can be hydrolyzed only with difficulty, and since they are present in the oils in only very small quantities, the use of even very acidic or very basic additions in the oil has substantially no effect on the adducts. Hydrocarbon oils containing the present antifoaming agents are stable when stored over long periods of time and also when subjected to heat and pressure conditions of engine and motor operation.

While the antifoaming effect of the acetal-ester adducts is obtained when they are employed in concentrations of up to 1.0% by weight, the adducts may be incorporated into hydrocarbon oils of much higher proportions, e. g., in amounts of up to 10 per cent or even 50 per cent of the weight of the hydrocarbon oil to give concentrates. Oils containing such high proportions of the adducts may be manufactured and sold for use as lubricant additives. Addition of small amounts of such concentrate to hydrocarbon oils may be made so as to supply an oil containing suitable quantities of the adducts.

Hydrocarbon oils which are rendered substantially antifoaming by incorporation therein of quantities of up to 1.0 per cent of the present adducts are synthetic or petroleum stocks of varying viscosities such as lubricating oils for internal combustion engines and motors, diesel fuels and lubricants and pressure transfer media, e. g., industrial lubricants, process oils, hydraulic oils, turbine oils, cutting oils, fluid greases, gear oils, shock absorber oils, spindle oils, journal bearing oils, pneumatic tool lubricants, etc. They may

be synthetic or natural hydrocarbons of any type, i. e., paraffinic, naphthenic or blended.

The invention is further illustrated, but not limited, by the following example.

*Example*

The antifoaming properties of lubricants may be determined according to the procedure generally described in Designation L-12-445 of the Coordinating Research Council, New York. Briefly this procedure involves bubbling air or an inert gas such as nitrogen through the hydrocarbon oil to be tested, employing standard apparatus and standard conditions.

The oil was placed in a standard 100-ml. graduated cylinder in the top of which was inserted a two-hole rubber stopper. An air-inlet tube extended through this stopper, to the bottom of which was attached a gas diffuser or porous stone sphere. The length of the inlet tube was adjusted so that when the apparatus was assembled, the sphere just touched the bottom of the cylinder. The sphere was attached to the inlet tube by means of litharge or glycerine, or by a copper tube soldered to the diffuser-stone coupling. The oil bath used was capable of controlling temperature at  $200^{\circ} \pm 10^{\circ}$  F. ( $93.3^{\circ} \pm 0.6^{\circ}$  C.), large enough to permit the cylinder to be immersed at least to the 90-ml. mark, and arranged to permit the visual observation of the graduations on the cylinder.

Dry nitrogen or air was supplied at the rate of 0.2 cubic foot per hour, employing a calibrated flowmeter. The sample was heated to  $120^{\circ}$  F. ( $48.9^{\circ}$  C.), and then cooled, before testing, to  $75^{\circ} \pm 5^{\circ}$  F. ( $23.9^{\circ} \pm 2.8^{\circ}$  C.) in a constant temperature room. 25 cc. of oil was used for each test.

With the air hose disconnected between the flowmeter and the delivery tube to the diffuser stone, the stone was allowed to soak in the oil for 5 minutes, at the end of which time the air flow (0.2 cu. ft. per hour) was started through the stone. Zero time was noted when the air or nitrogen bubbles started to rise from the stone. Readings of the top and bottom foam levels were taken at the end of a 5-minute period. The volume of foam was calculated from the two readings.

Employing the testing procedure described above there was determined the antifoaming effect of a liquid mixture of acetal-diethyl maleate adducts when added to a Champlin 30 SAE base oil in concentrations of from 0.02% to 0.05% by weight of the oil. The liquid mixture of adducts, B. P. above  $200^{\circ}$  C./0.6 mm.  $n_{D}^{25}$  1.4558 consisted of adducts of one mole of acetal with from 2 to 20 moles of diethyl maleate and was prepared by refluxing one mole of acetal (1,1-diethoxyethane) with 0.25 mole of diethyl maleate for 42 hours in the presence of a mixed free-radical promoting catalyst consisting of 1.0 cc. of tert-butyl peroxide and 1.5 g. of benzoyl peroxide, and separating from the resulting reaction mixture material boiling below the above-stated boiling point, as described in the previously cited copending application.

The following results were obtained:

| Concentration of adduct, weight percent | Foam, cc. |
|-----------------------------------------|-----------|
| 0.02                                    | 10 cc.    |
| 0.025                                   | 2 cc.     |
| 0.03                                    | none.     |
| 0.05                                    | none.     |

In the absence of an additive, the Champlin 30 SAE oil gave 71 cc. of foam under the same testing conditions.

Nonfoaming hydrocarbon oil compositions may be obtained by incorporating into such oils in a quantity of up to 1.0% based on the weight of the composition, other liquid mixtures of adducts of one mole of one of the present acetals with from 2 to 20 moles of the unsaturated dicarboxylates. Thus, instead of the acetal-diethyl maleate adducts employed in the above example there may be used, e. g., adducts of one mole of dimethoxymethane, of 1,1-(di-2-ethylhexoxy)-butane, of 1,1-dicyclohexoxybutane and of 1,1-diphenoxylheptane with from 2 to 20 moles of an ester such as di-n-butyl fumarate, diisoamyl maleate or di-n-octyl citraconate. The present adducts impart antifoaming properties to hydrocarbon oils, and may be used in the presence of other customarily employed additives such as extreme-pressure resisting additives, detergent additives, etc.

What I claim is:

1. A lubricant composition containing a hydrocarbon oil and up to 1.0 per cent by weight based on the weight of the composition of a liquid mixture of adducts having the formula



in which Y and Z are selected from the class consisting of hydrogen and the methyl radical and X is an alkyl radical of from 1 to 8 carbon atoms and n is an integer of from 2 to 20.

2. A lubricant composition containing a hydrocarbon oil and up to 1.0 per cent by weight based on the weight of the composition of a liquid mixture of adducts having the formula



in which X is an alkyl radical of from 1 to 8 carbon atoms and n is an integer of from 2 to 20.

3. A lubricant composition containing a hydrocarbon oil and up to 1.0 per cent by weight based on the weight of the composition of a liquid mixture of adducts having the formula



in which n is an integer of from 2 to 20.

JOSEPH E. FIELDS.

References Cited in the file of this patent

UNITED STATES PATENTS

| Number    | Name      | Date          |
|-----------|-----------|---------------|
| 2,380,304 | Gleason   | July 10, 1945 |
| 2,528,466 | Borsoff   | Oct. 31, 1950 |
| 2,528,465 | Borsoff   | Oct. 31, 1950 |
| 2,570,788 | Giammaria | Oct. 9, 1951  |

OTHER REFERENCES

Foaming of Aircraft-Engine Oils as a Problem in Colloid Chemistry, NACA Report ARR No. 4105, 1944, by McBain et al.